

## UNITED STATES PATENT OFFICE.

JEPHTHAH NEATH, OF STAINES, ENGLAND.

## CONSTRUCTION OF TENNIS COURTS.

No Drawing. Application filed September 8, 1925, Serial No. 55,412, and in Great Britain November 8, 1924.

This invention relates to the construction of tennis courts. More particularly, it relates to the construction of a form of hard court possessing many of the features of the usual clay court.

Although hard courts, as now built, have the advantage of not requiring frequent rolling and redressing, they nevertheless have the serious disadvantage of lacking the resiliency of clay courts. Various materials have been suggested for hard courts, including the use of common coal tar and asphaltum with pulverized materials of various forms. Coal tar and asphaltum, however, when mixed with pulverized materials, form a practically non-porous surface which after a rain dries only by slow evaporation, and which in consequence is quite slippery. In dry weather, the surface becomes hard and brittle and unyielding, and is very tiring to the feet of tennis players because of its lack of resiliency.

To prevent such difficulties and to produce a hard surfaced court possessing the advantages of a clay court, I employ a construction that is without the objectionable features formed in the use of coal tar or asphaltum. Instead of an impervious non-porous surface, I provide a porous surface through which rain and other moisture may easily percolate. As a result, the court does not become slippery and is fit for play after a wetting much sooner than if made of other materials. Furthermore, such a mixture as I employ possesses a resiliency which approaches that of a clay court, and which as a consequence is not as fatiguing as the usual form of hard court.

According to this invention water-gas tar is boiled and used as a binder for granulated or pulverized material such as spent oxide from gas purifiers, the mixture while hot, being spread over a foundation of clinker and coke breeze, a thin layer of brickdust or sand being then laid over the mixture and rolled until a hard firm surface is produced. The lines of the court can be marked with reinforced cement concrete.

In an example of the practical application of this invention, tar produced in water-gas making apparatus may be boiled and run into a receptacle containing spent oxide from gas purifiers in the proportions of 1 gallon of tar to 4 cwts. of spent oxide and

stirred to mix the ingredients. The ground being levelled and the clinker and coke breeze being spread thereon to a depth of 4 inches, double lines of wood are laid and filled in with cement, preferably reinforced by an iron bar running centrally of each pair of wood strips, the cement adhering to the clinker and coke breeze foundation. After the cement has set, the wood can be removed, and the spaces between the cement lines filled with the tar and oxide mixture to a depth of 1 inch, about 140 lbs. per square yard of the mixture being applied at a temperature of about 80 degrees Fahrenheit, and finally about 12 lbs. of brickdust or sand per square yard sprinkled over the top of the mixture. The court is then rolled until a hard firm surface is produced, when it is ready for immediate use, and does not require frequent rolling or re-dressing; its surface although dustless is porous, so that rain will quickly drain off it, and is resilient and not slippery, so that it is not so fatiguing to the players as are the usual hard courts.

Ordinary coal gas tar and bituminous mixtures have previously been used as binders for pulverized or granulated paving material, but the water-gas tar which I propose to use is a different substance and is not obtained from coal gas. It is composed of light oils, creosote oils, naphthalene and residual matters, and compared with coal gas tar it is of less density and less affected by changes of temperature. It is obtained by the following process:—Gas oil is distilled from crude petroleum, heated to about 300 degrees Fahrenheit, and sprayed into a vessel called a carbureter to enrich "blue" water gas contained therein. The enriched water gas is then passed from the carbureter to the gas washer, condenser, and tar extractor, in which latter the water gas tar is deposited.

The spent oxide herein mentioned is also a by-product of gas manufacture well known to gas engineers. This oxide which is used for absorbing sulphuretted hydrogen from gas is a "bog ore" rich in oxide of iron; it may contain for example 50 or 70 per cent of hydrated oxide of iron; it is placed in vessels called "purifiers" through which gas is passed, and when the oxide contains say 40 or 50 per cent of sulphuretted hydrogen,

it is removed and replaced by fresh oxide, the oxide removed being called "spent oxide."

What I claim and desire to secure by Letters Patent of the United States is:—

1. The construction of a tennis court of a mixture of boiled water-gas tar and spent oxide from gas purifiers.

2. The construction of a tennis court of a foundation of clinker and coke breeze, a <sup>10</sup> layer of a mixture of boiled water-gas tar with a material such as spent oxide from gas purifiers, and a thin upper layer of dry finely divided material such as brickdust or sand.

JEPHTHAH NEATH.